# EUROPEAN PATENT SPECIFICATION

(11) **EP 1 882 760 B1**
(45) Date of publication and mention of the grant of the patent: **05.01.2011**
(21) Application number: 07109809.9
(22) Date of filing: 07.06.2007
(51) Int. Cl.: D01F 2/08, D01D 1/10

(54) **Process for the production of flame-retardant viscose fibres**
Verfahren zur Herstellung von flammhemmenden Viskosefasern
Procédé pour la production de fibres de viscose ignifugées

(30) Priority: 28.07.2006 IT MI20061499
(43) Date of publication of application: 30.01.2008
(73) Proprietor: LENZING AKTIENGESELLSCHAFT, 4860 Lenzing (AT)
(72) Inventor: Tozzi-Spadoni, Francesco, 20124 Milano (IT); Seghizzi, Andrea, 20013 Magenta (Milano) (IT); Patritti, Giovanni, 28069 Trecate (Novara) (IT)
(74) Representative: De Gregori, Antonella

(56) References cited:
- DE-A1- 4 128 638
- FR-A- 2 138 400
- DATABASE WPI Derwent Publications Ltd., London, GB; AN 1980-04933C XP002480350 "Solution for forming self-stopping fibre" & SU 661 047 A (LESHCHINER A ET AL) 5 May 1979 (1979-05-05)
- DATABASE WPI Derwent Publications Ltd., London, GB; AN 1988-235439 XP002480129 & CS 8 609 247 A (PENCHAROVA I, BORODY M AND PAVLECH M) 15 June 1988 (1988-06-15)
- E.E. TREIBER: "Cellulose Chemistry and its Applications - Chapter 18: Formation of fibers from cellulose solutions" 1985, ELLIS HORWOOD LIMITED , CHICHESTER 131780 , XP002480100 ISBN: 0-85312-463-9 * page 465, lines 12-34 *
- A.G. WILKES: "Regenerated Cellulose Fibres - Chapter 3: The Viscose Process" 2001, WOODHEAD PUBLISHING LIMITED , CAMBRIDGE , XP002480101 ISBN: 1-85573-459-1 * paragraph [3.2.13] *
- M.S. CHOUDHARY, J.K. FINK AND K. LEDERER: "Investigation of the action of flame retardants in cellulose. I. Investigation of the flame retardant action of 2,2-oxybis(5,5-dimethyl-1,3,2-dioxaphospho rinane-2,2-disulfide) in cellulose" JOURNAL OF APPLIED POLYMER SCIENCE, vol. 30, no. 11, November 1985 (1985-11), pages 4345-4355, XP002479984

## Description

The present invention relates to a process for the production of flame-retardant viscose fibres.

In particular, the present invention relates to a process for producing a continuous multifilament viscose fibre having flame-retardant properties.

Viscose fibres, also called Rayon, are artificial fibres obtained starting from cellulose, a flammable substance of a vegetable origin.

Viscose fibres are obtained by the transformation of cellulose into a soluble derivative, sodium cellulose xanthogenate or xanthate, using a typical wet spinning process.

The production process is developed on batch or semi-batch plants and envisages the following main processing phases:

### - Wetting

In this phase soaking is effected with caustic soda (17-20%) to swell the fibres and form the cellulose alkali, enabling attack with respect to the alcoholic -OH and the dissolution of the hemicellulose:

Cell-OH + NaOH + H₂O = Cell-OH-NaOH-nH₂O

Cell-OH-NaOH-nH₂O = Cell --- ONa + n'H₂O

This reaction facilitates the development of the subsequent reactions.

### - Squeezing

In this phase the cellulose alkali is squeezed reducing the percentage of caustic soda which is recovered (IAC soda). - Disintegration and curing of the cellulose alkali.

The curing phase consists in a controlled demolition, of an oxidative nature, of the cellulose polymers, using the oxygen of the air to reduce the average polymerization degree of the cellulose. In order to guarantee the correct equilibrium between the optimum viscosity of the spinning solution and the textile characteristics of the fibre produced, it is important to keep the fundamental parameters such as time and temperature, under strict control.

### - Xanthation

In the xanthation phase gaseous carbon sulphide (CS₂) is added to the mass, which by reacting with the soda, forms the intermediate compound dithiocarbonate; this acts on the cellulose alkali giving rise to sodium cellulose xanthogenate.

Xanthogenate is a cellulose ester with dithiocarbonic acid (H₂OCS₂).

The reaction product of cellulose with the sulphide is not a homogeneous compound, the cellulose chains in fact initially have different esterification degrees, but after a time a redistribution takes place, which homogenizes the whole product.

At the end of the xanthation, the mass is discharged into the mixer where dissolution takes place under stirring, at a low temperature. At this point the liquid mass is finally "viscose", an orange-yellow-coloured liquid having a high viscosity and a penetrating odour due to the various sulphur compounds and elemental sulphur dissolved in the solution.

### - Curing of the viscose

The time period which precedes the spinning is called viscose curing. A polymeric and xanthic reassessment takes place in the liquid mass which leads to a reduction in the viscosity to a minimum value, and an increase in the instability of the xanthogenate, i.e. a greater tendency towards coagulation.

During the curing phase, which lasts 1-2 days, the viscose is subjected to other treatment necessary for improving its performance during extrusion.
- Elimination of the contaminants present as foreign particles, generally fragments of non-dissolved cellulose and common dirt.

This is normally effected in two filtering steps (1st filtration with Funda equipment, second filtration with filter presses), with increasing severity. -

### - De-aeration

This phase has the purpose of eliminating the air bubbles englobed and above all the air dissolved in the mass, whose presence is extremely dangerous during extrusion.

### - Spinning

During the spinning phase, the cellulose is regenerated from the viscose in fibrous form: at the outlet of the die hole the viscose encounters the coagulation bath which causes the coagulation of the viscose and hydrolysis of the xanthogenate. The filaments obtained under the stretching action in plastic phase are orientated and the yarn obtained then passes through various purification and preparation operations for subsequent uses.

Although the viscose fibres obtained according to the conventional techniques are applied in various sectors of the textile industry, they have the disadvantage of being easily flammable.

Attempts made for providing viscose fibres with flame-retardant characteristics have so far proved to be completely unsatisfactory.

These attempts are based on the "direct addition to the fibres" or "indirect addition to the solution" of alkaline viscose to be spun, of substances which inhibit or delay combustion, so-called flame-retardant additives.

As these substances are typically in solid and insoluble form, when they are applied as powders with a reduced particle-size directly to the yarn they have proved to be completely inappropriate for preventing combustion.

Furthermore, the addition of flame-retardant additives to the viscose mass to be spun causes a series of drawbacks mainly during the spinning phase. In most cases, a reduction has been observed, which can also be considerable, in the mechanical resistance properties of the yarn, above all when the dimensions are reduced.

One of the general objectives of the present invention therefore consists in providing a process for the production of a continuous viscose fibre having fire-resistance which can substantially reduce the drawbacks described above.

An objective of the invention consists in providing a process for the production of flame-retardant cellulose-based fibres which does not substantially jeopardize the mechanical resistance properties of the fibres themselves.

A further objective of the invention consists in providing means and operating procedures for producing a continuous viscose yarn having flame-retardant properties without changing its mechanical properties.

In view of these objectives, a first aspect of the present invention relates to a process for the production of cellulose-based fibres and in particular a continuous flame-retardant cellulose yarn, as disclosed in claim 1.

In general, the process according to an aspect of the invention comprises the addition of one or more flame-retardant additives belonging to the group of organophosphoric compounds to a cellulose viscose solution (cellulose xanthogenate) which limits:
- coagulation phenomena;
- the formation of a non-homogeneous dispersion which is incompatible with the subsequent spinning phase.

The Applicant has also found that the use of flame-retardant additives selected from organophosphoric compounds in particular having an average particle-size of about 10 microns, allows continuous flame-retardant fibres or yarns to be produced with good mechanical resistance characteristics. Among the group of organophosphoric additives which can be used within the scope of the invention, the compound 1,3,2-dioxaphosphorinan-2,2'-oxy-bis-(5,5-dimethyl-2-sulphide) has proved to be particularly suitable.

It has been found that this compound can be incorporated inside the structure of the viscose fibre without changing the fibre itself which would jeopardize the mechanical resistance properties even after continuous yarn spinning.

The Applicant has also found that by using a further specific flame-retardant additive combined with the organophosphoric additive, an improvement in the flame-retardant characteristics of the fibre is obtained.

In particular, particular advantages are obtained in terms of an increased flame-development resistance and a reduction in the production costs using a flame-retardant additive selected from tetrabromobisphenol A, sodium silicate and mixtures thereof, combined with said organophosphoric additive.

Tetrabromobisphenol A is known with the abbreviation TBBPA or the IUPAC name 2,2'6,6'-tetrabromo-4,4'-isopropylidendiphenol. As this compound is highly soluble in a strongly alkaline environment, such as that of the solution of cellulose xanthogenate, it does not interfere with the filtration process. During the washing phase with sulphuric acid, this additive reprecipitates in solid and insoluble form inside the yarn.

According to an embodiment this additive can be added until a percentage equal to 5% by weight with respect to the weight of the dry yarn, is reached.

Sodium silicate, the other additive which can be used in a combination with the organophosphoric compound, has the general formula Na₂O*n SiO₂. This compound is extremely soluble in water also at a high concentration forming high viscosity solutions, called liquid glass. Once it comes into contact with the washing acid (H₂SO₄), it also precipitates forming extremely insoluble SiO₂ and with a flame-retardant effect.

According to another aspect of the invention, the Applicant has found various specific operating conditions which allow a homogeneous dispersion to be obtained of the flame-retardant additive belonging to the group of organophosphoric compounds in a standard viscose solution (viscose xanthogenate) producing a continuous fire-resistant yarn.

The Applicant has observed that by mixing a dispersion containing a flame-retardant organophosphoric additive with a solution of cellulose xanthogenate inside a static mixer, a homogeneous dispersion of the additive is obtained within the solution of cellulose xanthogenate.

According to an embodiment, a solution containing one or more of the following solutions can be added to the mixture of the organophosphoric derivative:
- Solution in caustic soda of tetrabromobisphenol A (TBBPA). Although TBBPA is extremely insoluble in water, it has a certain solubility in caustic soda, typical of products belonging to the phenol group.
- Solution in water of sodium silicate.

The static mixer used typically comprises a series of mixing elements inserted inside a tube having a suitable length. 10-14 mixing elements are preferably adopted each comprising a short propeller rotated by 180° with alternating parts in the right and left area of the tube which has a length ranging from 800 to 1200 mm. Each element is aligned at 90° with respect to the subsequent element. The mixing propeller directs the flow of material radially towards the walls of the duct and backwards towards its centre. The inversion of the velocity direction and the division of the flow are the result of the combination of alternating elements situated at the inner sides of the duct which increase the mixing efficiency. The whole material is therefore completely and continuously mixed, eliminating radial temperature, velocity and composition gradients.

It has also been observed that a better homogeneity can be reached using a suitably made dynamic mixer instead of a static mixer, i.e. suitable for continuously mixing a high viscosity solution with a low viscosity solution/suspension.

In a subsequent phase, the dispersion produced in the static or dynamic mixer is subjected to filtration to allow the removal of the agglomerates of additive before the extrusion phase. The filtration is effected through at least two steps. The first filtration step typically envisages the use of a filter press with a filtrating septum capable of withholding particles having dimensions higher than 10 micrometer.

The second step comprises the use of a disk filter capable of withholding particles greater than 30 micrometer so as to remove possible coagulates formed which could block or slow down the subsequent extrusion.

The incorporation of these additives in the viscose fibre is effected following the formation process of a colloid previously described. In order to facilitate the dispersion operations, it is also appropriate for the additives to be predispersed (or dissolved) in water before being mixed with the viscose solution. The pre-dispersion (dissolution) of the additive in aqueous phase is conveniently effected inside a tank equipped with a stirring system. A suitable quantity of water is added to the tank in order to obtain an adequate concentration of solid, for example ranging from 10 to 20% by weight.

The aqueous pre-dispersion of additive is then transferred to the static mixer preferably using a dosage pump of the volumetric type. The flame-retardant additive is dosed so as to obtain an overall quantity not lower than 10%, preferably not lower than 15% by weight calculated with respect to the dry yarn.

The characteristics and advantages of a process for the production of flame-retardant viscose fibres according to the present invention will appear more evident from the following illustrative and non-limiting description, referring to the enclosed schematic drawing which illustrates an embodiment in five phases of the process of the invention.

With reference to figure 1, this shows an embodiment of the process which envisages the following phases:
a) predispersion/dissolution of the additive or additives in aqueous phase;
b) dosage of the predispersion in the solution of cellulose xanthogenate;
c) mixing process of the aqueous predispersion in the solution of cellulose xanthogenate;
d) filtration of the cellulose xanthogenate added. Said filtration is effected in two phases.
e) wet spinning to allow a spinning stability and good mechanical characteristics of the end-product.

In particular, in the predispersion phase a), a dispersion in water of a flame-retardant organophosphoric additive is charged into a tank 1 equipped with a suitable stirring system. The commercial dispersion is conveyed by a centrifugal pump 2 into the tank 4 passing through a cartridge filter 3 typically having dimensions of about 10 micrometer.

A effective dispersion of the additive is effected in the tank 4 by the addition of a suitable quantity of demineralized water, coming from a container 5, so as to obtain a final concentration of solid preferably ranging from 10 to 20% by weight.

The dosage of the additive is subsequently effected according to phase b) of the process. This phase avails of the use of a suitable dosage pump 6 which allows the removal and transferal of the predispersion into a colloidal solution of cellulose xanthogenate coming from the production process. The dosage pump 6 used is preferably of the volumetric type to guarantee precision and constancy of the dosage.

In order to have significant flame-retardant properties, the additive is present in a quantity preferably not lower than 10% calculated with respect to the dry yarn.

The subsequent phase c) of the process envisages mixing, inside a static mixer (or alternatively a dynamic mixer) 7, to obtain a homogeneous distribution of the predispersion of the flame-retardant additive in the solution of cellulose xanthogenate. The two liquids to be mixed have very different viscosities, and the mixer must therefore have a suitable length and geometry and must also be fed within a certain flow-rate range.

An ISG Motionless Mixer 3"x14 is preferably used. The ISG (Interfacial Surface Generator) comprises separate individual mixing elements inside the tube. The terminal part of the elements is produced so as to create a tetrahedral chamber with the adjacent element. Four holes passing through each element convey the flow; the holes are at oblique angles so that the material close to the walls of the tube is then sent towards the centre and, in the passage to the subsequent element, the flow is inverted from the centre towards the wall. This is therefore a radial mixing which eliminates the adhesion effect to the walls of the tube which may occur particularly in the mixing of more viscous fluids. Using this type of mixer 7, an optimum predispersion of the additive was obtained before passing to the subsequent filtration phase e).

In this phase, possible agglomerates of solid additive are removed before the extrusion process.

Phase d) is effected with the use of two filtration steps in series. The purpose of these filters is to drastically remove the agglomerates of materials formed after the action of the mixer.

The first filtration step typically envisages the use of a filter press 8 with a filtering septum capable of withholding the finer particles. The filtering unit conveniently comprises a filter press consisting of 8 filtering plates per 15 spinning rolls. Each plate is equipped with heavy Mako cloth + cellulose cloth from linters + rubberized cloth.

The purpose of the cards is to withhold agglomerates with dimensions greater than 10 micrometer: the density is 0.37 g/cm³, the basis weight 425 g/cm² and the thickness 1.15 mm.

The Applicant has observed that analogous results from the point of view of filtration degree and better results with respect to the duration and management of the plant can be obtained with the use of a self-cleaning filter such as a back-flow filter as illustrated in figure 2 enclosed. This filter, which typically does not require periodic filtration interventions, comprises a metallic net supported inside a metallic cylinder. The steel filtering net has a nominal dimension of the holes equal to 10 µm.

Once the filter has exhausted its filtering capacity, there is a device which is capable of "washing" the net using an aliquot of the filtered solution. This washing is effected on one section of the net at a time, so that the remaining sections can contemporaneously continue the filtering operation. The amount of solution used for the counter-washing is then disposed of separately.

This is followed by a second step on a nylon disk filter 9 with a capacity for withholding particulates having dimensions greater than 30 micrometer: the purpose of this filter is to block possible materials coming from lines or the press upstream following maintenance changes, etc.

The solution thus obtained allows a continuous acceptable spinning for longer than 15 days without significant problems of breakages, coagulations, titer reductions, etc.

The solution is then transferred to the die 10 for the spinning of a continuous flame-retardant viscose yarn.

During the spinning phase, the cellulose is generated from the viscose into a fibrous form: at the outlet of the die, the viscose (cellulose content about 8%) encounters the coagulation bath which causes the coagulation of the viscose and hydrolysis of the xanthogenate. The filaments obtained under the stretching action in plastic phase are orientated, and the yarn obtained then passes through various purification and preparation operations for the subsequent uses.

The dosage of the viscose is effected by means of spinning regulators (gear pumps); the dies are made of corrosion-resistant metals (alloys such as gold - platinum - iridium), with a number of holes of up to 200 (the number of holes is equivalent to the number of filaments of which the continuous fibre consists), with a diameter of the capillaries ranging from 50 to 200 µm; in addition to circular holes, the dies can have differently shaped holes to produce flat, trilobated filaments, etc.

The die is immersed in the coagulation bath, a saline solution having a high acidity which contains:
- Sulphuric acid
- Sodium sulphate and zinc sulphate, (slowing down the hydrolysis of the xanthic groups)
- Various modifiers (aliphatic and cyclic amines, polyoxyethyleneglycols, amides of oxyethylated fatty acids, etc, which facilitate extrusion, contact with the reagents and improve the stability of the xanthogenate during hydrolysis, etc.)

Contact with this bath at the outlet of the die hole neutralizes the alkalinity of the viscose, causing the immediate coagulation of the xanthogenate (no longer soluble in an acid environment) and hydrolysis, with demolition of the compound and by-products, loss of sulphur and consequent regeneration of the cellulose fibres.

This takes place progressively starting from the surface of the liquid thread which advances and penetrates inside until the whole filament is neutralized and coagulated.

In the meantime, the hydrolysis has also initiated and it is believed that in the first advance section of the thread, the xanthate has only decomposed to a fine surface layer, with the formation of a cuticle or skin. As the filament advances, the chemical reactions which regenerate the cellulose extend to the whole filament mass, from the outside (skin) to the inside (core).

It is possible to act on the composition of the bath to accelerate or delay the regeneration: in particular, zinc salts have a delaying action.

By increasing the content of these salts, filaments can be obtained with a preponderance of skin, whereas by reducing the percentage of zinc present, filaments in which the core prevails are obtained.

The skin is characterized by a more compact morphological structure, with more orientated fibres whereas the core has a less orientated fibrous structure. The delaying action of the zinc salt is due both to the lesser permeability of the skin formed in its presence, which therefore slows down the penetration, and also to the greater stability of the zinc xanthate with respect to sodium xanthate with a consequently slowing down of the decomposition.

The coagulation bath flows continuously fed by a recovery plant which continuously receives the return bath from the spinner. The exhausted bath has consumed part of the acid (used to neutralize the alkalinity of the viscose) and is enriched with salt (formed by the neutralization) and diluted with the water of the viscose; in addition to this it contains sulphurated products. The recovery comprises degasification, for the volatile sulphurated products, elimination of the excess salt as crystalline Na₂SO₄, elimination of the excess water by concentration and reintegration of the acid used up, in addition to a filtration.

During the regeneration, the yarn can be subjected to stretching, which produces the orientation of the cellulose chains modifying the morphological structure of the fibre, responsible for the textile characteristics of the product. In the classical process, the stretching and completion of the regeneration can be effected after the extrusion. In yarns for normal textile use, the average stretching is in the order of 10-50%, for yarns with special filaments it can also be much higher.

The viscose obtained has titers which vary from 60 den to 600 den. The fibre is continuous and multifilament. With the process of the invention, it is possible to produce both the shiny and opaque type, and dyed in mass in numerous colours. The mechanical properties of the continuous flame-retardant yarn obtained fall within the limits envisaged for standard products.

The main organophosphoric additive exerts its flame-retardant function inside the fibre, acting in solid phase, favouring the carbonization of the substrate and consequently slowing down flame propagation. The heated phosphorous reacts producing polymeric phosphoric acid, the latter causes the carbonization of the cellulose material with the formation of a vitreous layer which inhibits the pyrolysis mechanism, no longer fed by gaseous fuel. Furthermore, the intumescent layer protects the underlying polymer from the heat of the flame.

The secondary additives act according to the following mechanisms:
- the TBBPA acts in gas phase poisoning the flame, i.e. at the moment in which the substrate burns, it releases gases which slow down or inhibit the combustion process.
- the silicate, on the other hand, has an analogous mechanism to that of the organophosphoric compound, i.e. it facilitates the carbonization of the substrate (charring).

As viscose is a non-thermoplastic compound, when fabrics based on the fibre obtained with the process of the invention are subjected to free flames, they do not tend to melt, and are therefore not subject to the harmful effects to which fabrics produced with synthetic thermoplastic fibres such as nylon or polyester are subjected. When these materials are subjected to free flames, in fact, they tend to release incandescent drops which can propagate the fire, they also tend to shrink and create a hole in the fabric, thus annulling the protective function.

With the same mass, moreover, synthetic fibres release a much greater quantity of heat with respect to cellulose fibres.

An index which measures the facility with which a material burns is LOI (limiting oxygen index), it represents the minimum percentage of oxygen sufficient for maintaining combustion of the substance under examination. The greater the index, the lesser the tendency to burn will be.

Standard viscose has a LOI index of 18, the viscose containing additives obtained with the process of the invention has a LOI index conveniently ranging from 28-30.

The continuous flame-retardant viscose yarn of the invention, in titers of 220/46 and 330/56 has been tested in various national and foreign laboratories obtaining certifications. In particular, the viscose fabric of the invention has passed combustion tests according to BS5852 (1990).

As the flame-retardant additive remains dispersed inside the mass and as it is insoluble in water, the properties described do not deteriorate during the normal treatment to which the fibres are subjected during their processing and during the life of the end-product produced therewith (washing resistance).

The fibre and continuous yarn obtained with the process of the invention are applied in the textile industry for producing clothes, linings, outdoor knitwear and in furnishing for example in the production of fabrics for the covering of padding such as padded furniture, for protective clothing mixed with other intrinsically flame-retardant fibres or in drapery and curtaining mixed with other flame-retardant fabrics.

The fabric obtained with the process of the invention also has excellent transpirability and antistatic properties together with a good mixability with other fibres such as wool, acetate, silk, polyamide, linen and cotton.

The following example is provided for purely illustrative purposes of the present invention and should not be considered as limiting the protection scope as indicated in the enclosed claims.

### EXAMPLE 1

A fabric lining made of viscose according to the present invention was tested, having a weft of 300 den/0 20.5T/cm, a chain 300/400 23 yarns cm containing 15% by weight of 1,3,2 dioxaphosphorinan-2,2'-oxy-bis-(5,5-dimethyl-2-sulphide) calculated with respect to the dry yarn, coupled with a padding made of polyurethane NLTX 35F having the following characteristics: density 35 kg/m³, compression stress 3.3 kPa, tensile strength 80 kPa, elongation 100%, elastic yield 60% in accordance with the fire reaction group 1 IM.

When subjected to the UNI 9175 -9175/FA-1 test, the viscose lining proved to be inflammable after passing three series of tests.

## Claims

1. A process for the production of flame-retardant fibres or a continuous yarn based on viscose, comprising:
- mixing of a solution of cellulose xanthogenate with an aqueous dispersion of a flame-retardant organophosphoric additive in a mixer to obtain a homogeneous dispersion of said additive,
- filtration of the colloidal mixture formed to remove the solid coagulates formed,
- spinning of the filtered colloidal mixture through dies in a regenerating and coagulation bath, **characterized in that** the mixing phase is effected in a static or dynamic mixer and **in that** the filtration phase comprises a first filtration step in which particles with dimensions greater than 10 micrometer are withheld and a second step in which reformed particles or coagulates with dimensions greater than 30 micrometer are withheld.

2. The process according to claim 1, **characterized in that** said flame-retardant organophosphoric additive is 1,3,2-dioxaphosphorinan-2,2'-oxy-bis-(5,5-dimethyl-2-sulphide).

3. The process according to claim 1 or 2, **characterized in that** said organophosphoric additive is associated with at least another flame-retardant additive selected from the group comprising tetrabromobisphenol A, sodium silicate and mixtures thereof.

4. The process according to claim 1, **characterized in that** in said first filtration step a filter press or a self-cleaning filter is used and in the second filtration step a disk filter is used.

5. The process according to any of the previous claims 1-4, **characterized in that** it comprises a preliminary predispersion phase in water of the flame-retardant additive inside a tank equipped with a stirring system to obtain a total concentration of additive ranging from 10-20% by weight.

6. The process according to claim 5, **characterized in that** it comprises the dosing of the aqueous dispersion of the flame-retardant additives in the solution of cellulose xanthogenate so that said additives are present in a quantity not lower than 10%, preferably not lower than 15% by weight calculated with respect to the dry yarn.

7. A continuous fibre or yarn based on viscose with flame-retardant properties obtained by means of the process according to any of the previous claims 1-6.

8. The continuous viscose fibre or yarn according to claim 7, having a LOI index ranging from 28-30.

9. A continuous viscose fibre or yarn according to claim 7 having a total content of flame-retardant organophosphoric additive ranging from 10 to 20% by weight with respect to the dry yarn.

10. A textile article having fireproof properties comprising a continuous viscose fibre or yarn according to any of the claims 7-9.

11. The article according to claim 10, **characterized in that** it is selected from clothing items, linings, furniture coverings or padding, drapery or curtaining.

## Patentansprüche

1. Verfahren zur Produktion von flammhemmenden Fasern oder einem durchgehendem Garn basierend auf Viskose, umfassend:
- das Vermischen einer Lösung aus Zellulosexanthogenat mit einer wässrigen Dispersion eines flammhemmenden, organophosphorischen Zusatzstoffes in einem Mischer, um eine homogene Dispersion des Zusatzstoffes zu erhalten,
- das Filtrieren der gebildeten kolloidalen Mischung, um die gebildeten festen Koagulate zu entfernen,
- das Spinnen der gefilterten kolloidalen Mischung durch Gesenke in einem Regenerier- und Koagulationsbad, **dadurch gekennzeichnet, dass** die Vermischungsphase in einem statischen oder dynamischen Mischer erfolgt und das die Filtrierungsphase einen ersten Filtrierungsschritt umfasst, in dem Teilchen mit Maßen die größer als 10 Mikrometer sind, zurückgehalten werden sowie einem zweiten Schritt in dem umgeformte Teilchen oder Koagulate mit Maßen die größer als 30 Mikrometer sind, zurückgehalten werden.

2. Das Verfahren nach Anspruch 1, **dadurch gekennzeichnet, dass** der flammhemmende, organophosphorische Zusatzstoff 1,3,2-Dioxaphosphorinan-oxy-bis-(5,5-Dimethyl-2-Sulfid) ist.

3. Das Verfahren nach Anspruch 1 oder 2, **dadurch gekennzeichnet, dass** der organophosphorische Zusatzstoff mit mindestens einem weiteren flammhemmenden Zusatzstoff assoziiert ist der von der Gruppe ausgewählt ist, die Tetrabromobisphenol A, Natriumsilikat und Mischungen davon umfasst.

4. Das Verfahren nach Anspruch 1, **dadurch gekennzeichnet, dass** in dem ersten Filtrierungsschritt eine Filterpresse oder ein selbstreinigender Filter benutzt wird und im zweiten Filtrierungsschritt ein Scheibenfilter benutzt wird.

5. Das Verfahren nach einem der vorhergehenden Ansprüche 1 bis 4, **dadurch gekennzeichnet, dass** es eine vorbereitende Vordispensionsphase im Wasser des flammhemmenden Zusatzstoffs im Innern eines Behälters umfasst, der mit einer Rühreinrichtung ausgestattet ist, um eine Gesamtkonzentration des Zusatzstoffs zu erhalten die zwischen 10 bis 20% bezüglich des Gewichts liegt.

6. Das Verfahren nach Anspruch 5, **dadurch gekennzeichnet, dass** es die Dosierung der wässrigen Dispersion des flammhemmenden Zusatzstoffs in der Zellulosexanthogenatlösung umfasst, so das die Zusatzstoffe in einer Menge vorhanden sind die nicht niedriger als 10%, vorzugsweise nicht niedriger als 15%, ist bezüglich des Gewichts berechnet in Beziehung zum trockenen Garn.

7. Eine durchgehende Faser oder Garn basierend auf Viskose mit flammhemmenden Eigenschaften, erhalten mit Hilfe des Verfahrens nach einem der vorhergehenden Ansprüche 1 bis 6.

8. Die durchgehende Viskosefaser oder Garn nach Anspruch 7, mit einem Sauerstoffindex der zwischen 28 und 30 liegt.

9. Eine durchgehende Viskosefaser oder Garn nach Anspruch 7, mit einem Gesamtgehalt an flammhemmenden, organophosphorischen Zusatzstoff der zwischen 10 bis 20% bezüglich des Gewichts hinsichtlich des trockenen Garns liegt.

10. Ein Textilprodukt mit flammhemmenden Eigenschaften mit einer durchgehenden Viskosefaser oder Garn nach einem der vorhergehenden Ansprüche 7 bis 9.

11. Das Produkt nach Anspruch 10, **dadurch gekennzeichnet, dass** es von Kleidung, Futterstoffen, Verkleidungen oder Polsterungen für Möbel, Stoffladen oder Vorhängen ausgewählt ist.

## Revendications

1. Procédé pour la production de fibres ou d'un fil continu ignifugeants à base de viscose, comprenant :
- le mélange d'une solution de xanthogénate de cellulose avec une dispersion aqueuse d'un additif organophosphorique ignifugeant dans un mélangeur pour obtenir une dispersion homogène dudit additif,
- la filtration du mélange colloïdal formé pour éliminer les coagulations solides formées,
- le filage du mélange colloïdal filtré à travers des matrices dans un bain de régénération et coagulation, **caractérisé en ce que** la phase de mélange est effectuée dans un mélangeur statique ou dynamique et **en ce que** la phase de filtration comprend une première étape de filtration dans laquelle des particules avec des dimensions supérieures à 10 micromètres sont refusées et une deuxième étape dans laquelle des particules refusées ou coagulations avec des dimensions supérieures à 30 micromètres sont refusées.

2. Procédé selon la revendication 1, **caractérisé en ce que** ledit additif organophosphorique ignifugeant est le 1,3,2-dioxaphosphorinan-2,2'-oxy-bis-(5,5-diméthyle-2 sulfure).

3. Procédé selon la revendication 1 ou 2, **caractérisé en ce que** ledit additif organophosphorique est associé à au moins un autre additif ignifugeant sélectionnés parmi le groupe comprenant le tétrabromobisphénol A, le silicate de sodium ou des mélanges de ceux-ci.

4. Procédé selon la revendication 1, **caractérisé en ce que**, dans ladite première étape de filtration, une presse à filtre ou un filtre autonettoyant est utilisé et, dans la deuxième étape de filtration, un filtre à disque est utilisé.

5. Procédé selon l'une quelconque des revendications 1 à 4, **caractérisé en ce qu'**il comprend une phase de pré-dispersion préliminaire de l'additif ignifugeant dans l'eau à l'intérieur d'un réservoir équipé d'un système d'agitation pour obtenir une concentration totale d'additif dans la plage de 10 à 20% en poids.

6. Procédé selon la revendication 5, **caractérisé en ce qu'**il comprend le dosage de la dispersion aqueuse des additifs ignifugeants dans la solution de xanthogénate de cellulose de manière que lesdits additifs soient présents dans une quantité non inférieure à 10%, de préférence non inférieure à 15% en poids, calculée par rapport au fil sec.

7. Fibre ou fil continu à base de viscose avec des propriétés ignifugeantes, obtenu au moyen du procédé selon l'une quelconque des revendications 1 à 6.

8. Fibre ou fil continu de viscose selon la revendication 7, ayant un indice LOI dans la plage de 28 à 30.

9. Fibre ou fil continu de viscose selon la revendication 7, ayant une teneur totale d'additif organophosphorique ignifugeant dans la plage de 10 à 20% en poids par rapport au fil sec.

10. Article textile ayant des propriétés ignifugeantes comprenant une fibre ou fil continu de viscose selon l'une quelconque des revendications 7 à 9.

11. Article selon la revendication 10, **caractérisé en ce qu'**il est sélectionné parmi des articles vestimentaires, doublures, revêtements ou rembourrages de meubles, tentures ou rideaux.
